

## UNITED STATES PATENT OFFICE

2,338,710

## METHOD OF TREATING FIBROUS WEB MATERIAL

Lloyd L. Dodge, Wausau, Wis., assignor to National Paper and Chemical Company, Wausau, Wis., a corporation of Wisconsin

No Drawing. Application December 11, 1939,  
Serial No. 308,667

3 Claims. (Cl. 117—156)

This invention relates to the treatment of paper and like fibrous web material to enhance the desirable properties thereof, such as its wet strength, its resistance to penetration by moisture, grease and gases, and its resistance to alkali, acids and alcohol.

I have now found that the wet strength and other desirable properties of paper and similar fibrous web material can be materially increased by treating such paper and the like with an aqueous dispersion of a casein, a wax and a plasticizer, incorporating a methylene hardening agent into the treating composition and drying the treated paper or the like at an elevated temperature to harden the casein and fuse the particles of wax over the fibers. The treatment can suitably be effected during the course of manufacture of the fibrous web material, as by coating, spraying, immersing, or other form of application. Subsequent drying of the treated web on the usual driers of a paper machine, board machine or the like, is sufficient to give a finished product having the desirable properties above mentioned.

It is therefore an important object of this invention to provide a composition for application to paper and like fibrous web material for the purpose of increasing the wet strength of the paper, or enhancing other desirable properties such as those above enumerated.

It is a further important object of this invention to provide a method whereby paper and like fibrous web material, during the course of its manufacture, can be treated with an aqueous dispersion of a casein, wax, plasticizer and methylene hardening agent to increase its wet strength and impart other desirable properties to the fibrous web material.

It is a further important object of this invention to provide paper and other like material having increased wet strength and other desirable properties due to the treatment thereof with a composition including a hardened casein, a wax and a plasticizer.

Other and further important objects of this invention will become apparent from the following description and appended claims.

As already stated, the treating composition of my invention includes a casein, a wax and a plasticizer for paper, or cellulose fibers. The casein may be either a milk casein or a vegetable casein, such as may be obtained from oleaginous seeds. Animal protein is not satisfactory for my purpose. The term "casein" is therefore used in a generic sense to include both milk and vegetable

caseins. In the case of the vegetable casein, it is not necessary to employ a chemically isolated casein, since a substantially oil free, soybean meal, or flour, can be satisfactorily employed.

5 The wax to be used in my composition may suitably be in the form of a prepared wax emulsion, comprising a mixture of water, paraffin wax and emulsifier of the soap type. Such an aqueous emulsion of wax is obtainable under the trade name, "Paracol," but any stable aqueous wax emulsion may be used. Preferably, the wax particles in the emulsion have a maximum diameter of about 5 microns and a minimum diameter of about 1 micron, 80% of the particles averaging from  $2\frac{1}{2}$  to 3 microns in diameter. The total solid content of such an emulsion is usually in the neighborhood of 50%. The emulsifier may be any of the known emulsifying agents, such as ethanol amine esters of higher fatty acids, saponified fatty acids, and the like. The pH of the wax emulsion is, in general, about 7, or slightly under 7, but quite a wide range is permissible.

10 Of the plasticizers for cellulose fibers that I have found to be suitable, polyhydric alcohols, such as glycerol and the water soluble glycols, sugars, deliquescent salts, and the like, may be mentioned. A preferred plasticizing composition is prepared from 1 part of glycerol and 2 parts of corn sugar by weight. The plasticizer is primarily selected because of its ability to plasticize the fibers and not for the purpose of plasticizing the casein, although the latter is also realized.

15 The following will serve to illustrate a preferred embodiment of my invention, parts by weight being given except where otherwise specified:

Example

20 To 55 parts of casein are added 500 parts of water containing 5 parts of dissolved borax. The aqueous mass is heated to  $180^{\circ}$  F. and stirred until a clear dispersion of the casein is obtained. There are then added 25 parts of a plasticizer comprising a mixture of glycerol and corn sugar, 10 parts of the previously described wax emulsion having a 50% solid content, and 5 parts of a 6% aqueous solution of formaldehyde. After the mixture has been thoroughly agitated and a uniform dispersion obtained, it may suitably be diluted with an equal volume of water before use. Such dilution brings the solid content from about 14% to about 7%.

25 A considerable variation in the proportions of the ingredients of my composition is permissible. For instance, on the basis of the casein, the proportion of solids in the wax emulsion may be be-

tween 2 and 25% by weight of the casein, and the proportion of plasticizer between 10 and 100% by weight of the casein. By increasing the proportion of wax, greater transparency is obtained in the final sheet.

In place of borax, any suitable alkaline substance may be used for the dispersion of the casein. If soybean casein, or soybean flour be substituted for animal casein, a somewhat higher degree of alkalinity is necessary to effect a uniform dispersion of the vegetable caseins and for this purpose caustic alkali, either by itself or with a small proportion of calcium hydroxide, may be used.

The amount of formaldehyde may also be varied, depending upon the degree to which the casein is to be hardened or insolubilized. Other methylene hardening agents, such as hexamethylene tetramine, may be used in place of formaldehyde, or polymers of formaldehyde may be used. Instead of incorporating the methylene hardening agent directly in the aqueous treating composition, the fibrous material, after treatment with the aqueous emulsion, may be subjected to formaldehyde gases. It is preferable to incorporate the formaldehyde into the aqueous treating composition just prior to its use, since otherwise coagulation is likely to take place.

In the treatment of paper on the paper machine to increase its wet strength, the aqueous treating composition may best be applied at a size press intermediate sections of the driers at which point the moisture content of the sheet is less than 30%. Either one or both sides of the paper may be contacted with the aqueous treating composition. The treated paper is then run immediately over the driers beyond the point of application of the aqueous treating composition to dry the paper quickly, insolubilize the casein and cause the wax to fuse over the fibers of the paper. The penetration of the wax into the paper is very slight, but the plasticizer, being water soluble, penetrates quickly and completely into the body of the sheet.

While my invention is applicable to various kinds and weights of paper, as well as to paper board and the like, it finds particular application in the case of light weight wrapping papers, vegetable parchment and the like, for use in the wrapping of fats, such as lard, candies, and the like.

By way of example, if a paper of 30 lbs. basis weight per ream of 500 sheets, each 24 x 36 inches, is treated in accordance with the method just described, the increase in weight due to retained solids is approximately 1 lb. per ream. The sheet becomes much more dense, the pin holes being largely closed by the retained solids, and therefore much more resistant to penetration by air, grease and moisture. The treated paper will also be found to be a much better protection for foodstuffs against the formation of mold and against the development of rancidity, than a paper not so treated.

A particularly important application of my aqueous treating composition is found in the treatment of light weight wrapping papers formed from a relatively free stock, that is, a stock that has not been well hydrated. Owing to the openness of such a sheet, the aqueous treat-

ing composition need be applied only to one side of the sheet to effect a thorough impregnation thereof. The treated paper has a greatly increased wet strength and is relatively moisture-, grease-, and gas-proof despite the comparatively open formation of the sheet itself. Light weight wrapping papers of kraft pulp as well as sulphite pulp may be treated in this manner.

One of the important features of my invention 10 is the incorporation of the plasticizer in the casein-wax emulsion, since this is largely responsible for the superiority of my coating composition. The grease-proofness of the paper due to the casein-wax content is not adversely affected 15 by the presence of the plasticizer, while the paper is thoroughly plasticized. Ordinary wax coatings are likely to be broken by severe creasing, thereby destroying or greatly reducing the grease-proofness of the coated sheet. In the case 20 of my plasticized, casein-wax coated paper, creasing of the coated paper, has no such effect since the coating remains intact. The same result is not obtained by separately plasticizing the body 25 of the fibrous web material and then applying an unplasticized casein-wax coating thereover.

It will, of course, be understood that various 30 details of the process may be varied through a wide range without departing from the principles of this invention and it is, therefore, not the purpose to limit the patent granted hereon otherwise than necessitated by the scope of the appended claims.

I claim as my invention:

1. In a method of making paper comprising 35 the steps of forming a wet paper web and heating the web to dry the same, the improvement including simultaneously applying to said wet paper web a coating of an aqueous dispersion of a protein selected from the class consisting of casein 40 and the water insoluble proteins naturally present in oleaginous seed material, paraffin wax, a plasticizer and a methylene containing hardening agent, whereby said web on subsequent heating is rendered stronger and more proof to moisture, 45 grease and gas due to resulting hardening of the protein and fusion of the wax on the paper fibers.

2. In a method of making paper comprising the 50 steps of forming a wet paper web and heating the web to dry the same, the improvement including simultaneously applying to said wet paper web a coating of an aqueous dispersion of soya bean protein, paraffin wax, a plasticizer and a methylene containing hardening agent, whereby 55 said web on subsequent heating is rendered stronger and more proof to moisture, grease and gas due to resulting hardening of the soya bean protein and fusion of the wax on the paper fibers.

3. In a method of making paper comprising the 60 steps of forming a wet paper web and heating the web to dry the same, the improvement including simultaneously applying to said wet paper web a coating of an aqueous dispersing of casein, paraffin wax, a plasticizer and a methylene 65 containing hardening agent, whereby said web on subsequent hardening is rendered stronger and more proof to moisture, grease and gas due to resulting hardening of the casein and fusion of the wax on the paper fibers.